

Sept. 27, 1949.

H. W. HALL

2,483,198

METHOD OF TREATMENT OF LIGNO-CELLULOSIC MATERIAL  
AND PRODUCT RESULTING THEREFROM

Filed March 16, 1943

*Fig. 1*



*Fig. 2*



*Fig. 3*



*Fig. 4*



*Fig. 5*



*Fig. 6*



INVENTOR.

Horace W. Hall  
Harold E. Cole

ATTORNEY

## UNITED STATES PATENT OFFICE

2,483,198

METHOD OF TREATMENT OF LIGNO-CELLULO-  
SIC MATERIAL AND PRODUCT RESULT-  
ING THEREFROM

Horace W. Hall, Newton, Mass.

Application March 16, 1943, Serial No. 479,386

3 Claims. (Cl. 8—115.6)

RELEVANT FIGURE 1

This invention relates to the treatment of woods and other ligno-cellulosic substances, including vegetable cane fiber, with materials to render them fire resistant, water-proof and denser and harder than the normal state of such woods and the like.

One object is to make a highly fire-resistant article and good heat-insulator at a relatively low cost by using an inexpensive base or foundation board and impregnating a surface portion with an adhesive and fire-proof material that chemically re-acts therewith. Another object is to make said article in the form of a panel or other finished product, if desired, having a mottled design inherent in the surface that is made simultaneously with the article itself, the form of which can be varied considerably by what is done during the process of manufacture.

The finished article is a chemical re-action product of the materials entering into it having a surface portion that is non-combustible and an extraordinarily efficient heat insulator, yet hard and capable of taking high finish.

The foregoing and other objects which will appear as the nature of the invention is better understood, may be accomplished by a construction and process such as is disclosed by the drawings and specification. The nature of the invention is such as to render it susceptible to various changes and modifications, and, therefore, I am not to be limited to said disclosures; but am entitled to all such changes therefrom as fall within the scope of my claims.

In the drawings:

Figure 1 is a perspective view of the material to be impregnated. Figure 2 is a similar view after the adhesive has been applied to said material and Figure 3 is a similar view after the rock wool has been applied to said adhesive.

Figure 4 is a front elevational view showing the impregnated article under pressure between two iron plates.

Figure 5 is a front elevational view showing the said article under pressure and with heat being applied to it.

Figure 6 is a perspective view of my finished product showing the mottled effect achieved on the surface.

Reference is made to my Patent No. 2,366,025 issued December 26, 1944, because the invention herein disclosed is in part, another development of the disclosure in that application; but producing among other things a superior, non-heat

conducting article and one that is less brittle, but tougher.

My process may be illustrated by the treatment of a piece of material 10 made of vegetable cane fiber such as sugar cane fiber, which is relatively soft. There are various ligno-cellulosic materials available which may be in the form of wood, composition board and the like. Moisture content should preferably not exceed 10 to 12%.

I apply urea formaldehyde resin glue 11 liberally to the surface of the article to be treated. Said glue 11 is preferably freshly mixed and it could have a cold setting catalyst for quicker dehydration in the preliminary process, although that is not necessary. Said glue penetrates into the cellular structure of said piece. One ounce of glue to a square foot of the surface area to be covered would be a suitable amount. After about fifteen minutes, if no catalyst was previously used, another coat of glue in about the same quantity should be applied with or without some well known curative catalyst, and while it is still wet, rock wool 12 or other mineral wool is applied to the wet surface at once. Said rock wool 12 is applied in quantity thick enough to absorb the free moisture of the glue so that the surface being coated is substantially dry. It is preferable to apply two coats of said glue 11 as described; but not necessary. Much depends upon the depth of penetration and thickness of fire-proof surface portion desired. Phenol formaldehyde or other material which chemically reacts and bonds with the ligno-cellulosic fibers and 35 with rock wool, may be used.

Smooth steel plates 14, waxed to keep them from sticking should be placed on the surfaces of the piece being treated since both surfaces are usually treated. The article is thus cold 40 pressed between the plates with pressure sufficient to establish uniform capillarity throughout the treated portion. This pressure is preferably maintained for a substantial period of time, such as two days, for diffusion of the adhesive 45 impregnate into the cellulosic structure of the rock wool and the treated portion of the ligno-cellulosic material. The surface coating is now somewhat soft, but smooth and dry; but not waterproof, although quite fire-proof on the surface, 50 at least, where the rock wool is located.

The coated piece is now pressed between two hot plates 16, heated by heating elements 17 and properly waxed to prevent sticking, at temperatures of 250 to 350 degrees F. for 20 to 30 minutes 55 with a greater pressure than before, preferably

from 150 to 250 pounds to the square inch. Plasticization of the rock wool and impregnated portion of the ligno-cellulosic material with the impregnate occurs in about 5 minutes followed by a final chemical curing and hardening of said coating materials with the treated cells of the ligno-cellulosic material into an irreversibly bonded and integral coating in the finished article which can be nailed, screwed and is generally workable.

When an attractive design is desired on the surface of the finished product, the rock wool or other mineral wool, or asbestos, is placed on said urea formaldehyde glue in matted thin layers or other sheet form preferably varying in thickness, instead of in powdered form or small fibers. The solid sheets even though small, give the finished product a mottled design, whereas if small particles of powdered mineral wool or the like is used the finish will be quite plain and uniform. Of course, various color effects can be attained by using well known coloring matter in the materials applied to the surface. Different designs are achieved by different sizes and shapes of said sheets, and by spacing them apart.

Any glue that reacts with rock wool or other mineral wool or asbestos is suitable provided it is capable of impregnating and entering into proper chemical reaction with the ligno-cellulose article. Also rock wool and asbestos could be used together if desired as they both react with the urea formaldehyde glue.

What I claim is:

1. A method of manufacture comprising applying urea formaldehyde glue to the surface of ligno-cellulosic material, then applying rock wool to said glue on said surface, then applying pressure to said surface and then applying heat and greater pressure thereto until said material, glue and wool chemically react.

2. A method of manufacture comprising applying urea formaldehyde glue to the surface of ligno-cellulosic material, allowing said glue to set, then applying more of said glue to said surface and while it is still wet applying rock wool thereto sufficient to present a dry surface, then applying pressure and heat to said surface until said material, glue and wool chemically react.

3. A manufactured product comprising cellulosic material the surface portion of which is impregnated with urea formaldehyde glue and outside of which is the hardened chemical reaction product of said glue and rock wool.

HORACE W. HALL.

#### REFERENCES CITED

The following references are of record in the file of this patent:

#### UNITED STATES PATENTS

| Number    | Name             | Date          |
|-----------|------------------|---------------|
| 4,688,420 | Kelly            | Dec. 10, 1901 |
| 885,376   | Ray              | Apr. 21, 1908 |
| 1,284,296 | Frederick        | Nov. 12, 1918 |
| 1,370,023 | Kempton          | Mar. 1, 1921  |
| 1,589,094 | Barringer et al. | June 15, 1926 |
| 1,796,631 | Stryker et al.   | Mar. 17, 1931 |
| 2,021,348 | Beckwith et al.  | Nov. 19, 1935 |
| 2,252,157 | Bergin et al.    | Aug. 12, 1941 |
| 2,366,025 | Hall             | Dec. 26, 1944 |

#### FOREIGN PATENTS

| Number | Country       | Date |
|--------|---------------|------|
| 8,081  | Great Britain | 1884 |

#### OTHER REFERENCES

Chem. & Met. Eng., April 1932 (vol. 39, No. 4), pages 219-221. (Copy in Division 55.)